

April 28, 1936.

E. C. DOMM

2,039,067

COPPER ANTIMONY OR COPPER BISMUTH COATED FERROUS METALS

Filed July 8, 1935



Inventor:  
Elgin Carleton Domm,  
By Drydenforth, Lee, Chittor & Niles,  
Attys.

## UNITED STATES PATENT OFFICE

2,039,067

COPPER-ANTIMONY OR COPPER-BISMUTH  
COATED FERROUS METALSElgin Carleton Domm, Niles, Mich., assignor to  
National-Standard Company, Niles, Mich., a  
corporation of Michigan

Application July 8, 1935, Serial No. 30,339

20 Claims. (CL 91—68.2)

This invention relates to copper-coated ferrous metals and a method of preparing them, and more particularly to rubber-coated ferrous objects having copper-antimony, copper-arsenic or copper-bismuth undercoatings.

In the production of steel objects, and particularly objects which are to be rubber-coated, it is necessary to secure very great adhesion to rubber. It has hitherto been attempted to electroplate alloys directly upon ferrous objects, but this presents extreme difficulties, inasmuch as it is essential to maintain the current density without the slightest variation. In connection with irregularly shaped articles such as motor mounts, in which the utmost in adhesion is required, such uniformity is not obtainable by this method.

It has now been discovered that a ferrous object may be plated with copper, and then may be plated with a thin coating of arsenic antimony or bismuth thereon. While neither the copper nor the arsenic antimony or bismuth have any substantial adherence to rubber by themselves, the copper and antimony, copper and arsenic, and copper and bismuth, when plated separately upon each other, affect each other in some way, presumably by alloying, so that the metals, when rubber is vulcanized thereon, give tremendous adherence thereto. Motor mounts so treated show an adherence sufficient to resist a stress of from 300 lbs. to over 600 lbs. per square inch without tearing. As a matter of fact, the rubber will often be found to rupture within itself rather than to pull loose from the metal.

In accordance with the invention, a ferrous object, such as a motor mount 1, which is illustrated diagrammatically in broken section in the drawing, is electroplated with a thin coating of copper 2, and a thin coating of arsenic antimony or bismuth 3 is then plated thereon, after which a rubber coat 4 is vulcanized thereto. The deposition of the metals may be accomplished by electroplating, but it is preferred to treat the ferrous object with an acidified solution of copper sulfate, whereby copper deposition is secured by ionic displacement. A satisfactory solution for this purpose may be prepared in the proportions of 3 oz. copper sulfate, 1 gallon of water, and 1/5 gallon of muriatic acid. The ferrous object is first cleaned, as by acid, sand-paper or sand-blast, and is then dipped into the solution for 1-2 seconds, after which it is rinsed in cold water. A thin coating of metal of the class consisting of arsenic, antimony and bismuth may then be electroplated upon the copper. It is preferred to plate by substitution of such metal for a por-

tion of the copper by displacement from a solution of an appropriate electrolyte. In the case of antimony, a satisfactory electrolyte may be prepared by dissolving 4 oz. of antimony trichloride in a mixture of 2 gallons of hydrochloric acid (40%) and 8 gallons of water. The article is immersed in this solution for a period of 1 to 3 seconds and is then given a cold water rinse. It is then promptly dried to prevent corrosion. Preferably, the drying is carried out by immersion for a few seconds in a bath of boiling water, after which air-drying will take place rapidly enough to prevent corrosion.

In the case of bismuth, a satisfactory solution may be prepared in the proportions of 2 oz. of sodium bismuthate, 2 oz. sodium chloride, 1/2 gallon concentrated muriatic acid and 1/2 gallon of warm water. The solution is thoroughly mixed and is then ready for use. The article may be immersed from 3-10 seconds, and is then treated as in the case of the antimony-coated article.

In the case of arsenic, it is preferred to plate by substitution of arsenic for a portion of the copper, by displacement from a solution of an arsenic electrolyte. A satisfactory solution may be prepared from 3 oz. of sodium cyanide, 1/2 oz. red sulfide of arsenic, and 1 gallon of water. The copper-coated object is then dipped in the solution for a period of the order of one second, after which it is rinsed in cold water and then rapidly dried. The arsenic coating oxidizes with extreme rapidity and in order to prevent this, it is preferred to immerse the object in boiling water for a few seconds, say three seconds or more, and then dry it, the heat of the water causing the drying to occur rapidly enough to avoid corrosion.

It has been discovered that the concentration of the baths may vary within rather wide limits without affecting the rate of deposition of either the copper, antimony or bismuth. For example, the copper content may vary from 9 to 16 grams per liter, the arsenic from .1 to .45 gram per liter, the antimony from 10 grams to 20 grams per liter, and the bismuth from 7.5 to 15 grams per liter with no substantial variation in the rate of deposition. Immersion of a ferrous article as described will produce a uniform copper coating of .002 to .007 oz. of copper per square foot of area, the arsenic will plate a uniform coating of about .001 to .005 ounce per square foot, the antimony bath will plate a uniform coating of about .005 oz. of antimony per square foot, and the bismuth solution will be of the order of .001 oz. of bismuth per square foot of surface.

Following the plating treatment, the ferrous object is coated with rubber which is then vulcanized. In each case the use of a copper under-coat produces many times the adherence to rubber brought about by the use of the metal without the under-coat.

As used in this application, the term "electroplating" denotes any form of coating by electricity, whereas "electrodeposition" is used to denote ionic displacement. The rubber used for the coating material may be any suitable form of rubber, and these are well known to those skilled in the art.

The foregoing detailed description has been given for clearness of understanding only, and no unnecessary limitations should be understood therefrom, but the appended claims should be construed as broadly as permissible, in view of the prior art.

This application is a continuation in part of my copending application Ser. No. 706,736 filed January 15, 1934.

What I claim as new, and desire to secure by Letters Patent, is:

- 25 1. The method of producing a highly rubber adherent ferrous base object which comprises plating a thin layer of substantially pure copper thereon, and electroplating a layer of metal of the class consisting of arsenic, antimony and bismuth thereon, the layer being thin enough to alloy throughout with the copper under atmospheric temperature or the temperature of vulcanization, and adherently vulcanizing a coating of rubber thereto.
- 30 2. The method as set forth in claim 1, in which the second metal is arsenic.
- 35 3. The method as set forth in claim 1, in which the second metal is bismuth.
- 40 4. The method as set forth in claim 1, in which the second metal is antimony.
- 45 5. The method as set forth in claim 1, in which the thickness of the copper is of the order of .002 to .007 ounce per square foot of area.
- 50 6. The method as set forth in claim 1, in which the thickness of the arsenic antimony or bismuth is of the order of .001 to .005 ounce per square foot of surface.
- 55 7. The method as set forth in claim 1, in which the thickness of the copper is of the order of .002 to .007, and of the arsenic, antimony or bismuth is of the order of .001 to .005 ounce per square foot of area.
- 60 8. The method of claim 1, in which the double plated object, while still wet, is immersed in hot water, whereby it is rapidly dried without corrosion.
- 65 9. A ferrous highly rubber adherent base object comprising a ferrous base, a thin substantially pure copper layer thereon, a layer of metal of the class consisting of arsenic, antimony and bismuth on the copper, the layer being thin enough to alloy throughout with the copper under

atmospheric temperature or the temperature of vulcanization, and a layer of rubber adherently vulcanized thereto.

10. A ferrous base object as in claim 9, in which the second metal is arsenic.

11. A ferrous base object as in claim 9, in which the second metal is antimony.

12. A ferrous base object as in claim 9, in which the second metal is bismuth.

13. An object as in claim 9, in which the object is a steel motor mount, and in which the thickness of the arsenic antimony or bismuth layer is of the order of .001 to .005 ounce per square foot of area.

14. An article as set forth in claim 9, in which the thickness of copper is of the order of .002 to .007 ounce per square foot of area.

15. An article as set forth in claim 9, in which the thickness of the arsenic antimony or bismuth is of the order of .001 to .005 ounce per square foot of surface.

16. An article as set forth in claim 9, in which the thickness of the copper is of the order of .002 to .007 and of the arsenic antimony or bismuth is of the order of .001 to .005 ounce per square foot of area.

17. The method of producing a highly rubber adherent ferrous base object which comprises electroplating a thin layer of substantially pure copper thereon, and electrodepositing a layer of metal of the class consisting of arsenic, antimony and bismuth thereon, the layer being thin enough to alloy throughout with the copper under atmospheric temperature or the temperature of vulcanization, and adherently vulcanizing a coating of rubber thereto.

18. The method of producing a highly rubber adherent ferrous base object which comprises electrodepositing a thin layer of substantially pure copper thereon, and electrodepositing a layer of metal of the class consisting of arsenic, antimony and bismuth thereon, the layer being thin enough to alloy throughout with the copper under atmospheric temperature or the temperature of vulcanization, and adherently vulcanizing a coating of rubber thereto.

19. The method of producing a highly rubber adherent ferrous base object which comprises electrodepositing a thin layer of substantially pure copper thereon, and electrodepositing a layer of metal of the class consisting of arsenic, antimony and bismuth thereon, the layer being thin enough to alloy throughout with the copper under atmospheric temperature or the temperature of vulcanization.

20. A ferrous base object comprising a ferrous base, a thin substantially pure copper layer thereon, a layer of metal of the class consisting of arsenic, antimony and bismuth on the copper, the layer being thin enough to alloy throughout with the copper under atmospheric temperature.

ELGIN CARLETON DOMM.